

## UNITED STATES PATENT OFFICE

2,411,580

## CONTAINER WALL

Willard O. Manor, Monroe, Mich., assignor to  
 Consolidated Paper Company, Monroe, Mich., a  
 corporation of Michigan

No Drawing. Application September 30, 1943,  
 Serial No. 504,383

1 Claim. (Cl. 117—82)

1

This invention relates to shielding, protecting and coating walls, more particularly of fiber-like containers.

This invention has utility when incorporated in methods of compounding and applying, and also in ingredients of compositions and their association, especially with reference to fiber types of containers with an undercoating for a barrier between the contents and the wall. The primary course herein is laying of a thin film, desirably of elastic or stretchable properties having toughness in maintaining a skin upon a container wall or undercoating.

The skin and undercoating may serve as a responsive severing means to effect isolation between the wall and contents. The container proper may be, in its use, not primarily for refill service. In such latter instances the material may be fiber developed from rag, paper, grass, straw, or wood pulp, and compositions therewith, in the general class of fiber board, paper board, box board, and the like.

As to the coatings or coating materials, special value has been developed in features of toughness or elasticity. In this type of compressible fiber board stock, such is frequently blanked out and sent in knocked-down shape to be built up into containers. In this blanking, there may be scoring and marking or cutting. Under this invention the coating may be applied at or before the blanking operation and be efficient in the assembly of the blank into a container even as to the corners where there has been scoring or folding. The purpose of the coating is to isolate the charged contents or material from attacking the container. The contents may be hygroscopic, a solvent, vapor, grease or oil.

Additional problems arise in the handling of hot substances. The substance to be placed in the container may have seemingly no affinity for the container, or be readily fracturable therefrom, as paraffine wax. Again, it may be a substance having tacky or adhesive traits as asphalt. The contents of the container as reposing or solidifying may or may not tend to hold the container to shape. Should such contents normally tend not to hold to shape, the container adopted hereunder may be of such physical strength in its container walls as to be effective for such holding to shape.

With 50% starch, as Casava, there may be an equal quantity, or 50% of a film-forming chemical. These are in the fields of resins, or resin-like materials, and in the cellulose group from polyvinyl alcohol and including methyl cellulose. In this compounding, referred to as equal quantities, there may be a variation in the starchy substances of as much as one-half, and up to 100% of the film-forming material without starch. The traits to be considered are those of economy.

5 for the purpose sought. In this build-up for the solids of the starch and film-forming plastic, such may be 7# each with say 200# of water. This thin gruel direct water solution, desirably as a batch, may have a tempering, or water-holding trait or softness characteristic imparted thereto by some 20# of glycerine. The pliancy or softness in achieving this nondrying factor for this tough characteristic may be attained for the plastic of the coating composition by the use, in lieu of glycerine, of di-ethylene glycol, tri-ethylene glycol, or sulfonated oil, say of the castor type. This proportion of the tempering agent, when in the region of 20# in the 214# proportion suggested, is of commercial economy. However, as there may be longer storage period or other factors, such as the character of the calendering or facing for the fiber, variation may be adopted. In fact, as much as 40# of tempering agent or plasticizer has been used.

10 This composition of starch, plastic and tempering agent, has but slight absorption properties as to penetration of the fiber board or wall to be coated. It has non-crumbling properties of viscosity as well as retained elasticity effective as the tempering is a property thereof. In practice, it seems to extend as a very thin film or skin. The extent thereof in applying, whether by spray, brush, dipping or roll coating, may be only just sufficient to effect the continuity for such coating.

15 This film coating continuity is an isolating agent effecting dissipating of attack upon the wall due to the contents. In the instance of severing from the contents, when of a non-tacky nature, altho molten or at a high temperature as filled into the container, the coating may to a major extent go with the wall, instead of adhering with or becoming a part of the contents. In the instance that the contents are edible, these are matters to be given attention. However, due to the very thin character of this film, it is of such incredibly minor proportion as to be not in the realm for consideration as an adulterant or contamination of the container contents when, in removal, this film be associated with such contents.

20 Efficient isolation between the container and its contents is achieved by locating this stretchable film on an undercoating. The undercoating cooperates as a dam or barrier comprising a dispersion of a powder-like material, preferably very fine and to have it effective in continuity. However, efficient results in the non-food field have been obtained with fine clays or silicates, such as 25 kaolin. This undercoating is wiped, laid, sprayed or rolled, say in association with water or a glue agent, and thereby anchored through the action of this film-carrying overcoating.

20 Instead of elementally handling this undercoating as merely the kaolin and the glue and

water vehicle therefor, supplemental traits of advantage may be achieved in efficient dispersion thru the medium of a low grade karaya gum of high viscosity. This gum has been used in quantities and range from 5 3/4# to 7#. In fact, instead of this karaya gum, gum arabic or gum tragacanth may answer; but commercially there has been advantage in the karaya type. This advantage arises from its great rate of water solubility. With a charge or quantity of gum, there may be mixed therewith a carbonate. For this solution there may be 150# of water. The carbonate, when an ammonium bicarbonate, seems among the carbonates to contribute to a greater extent in smoothing out the mix and holding such for a maintained high degree of fluidity. This proportion for the carbonate may be taken as 13 3/4#. At times there are variations in the gum, and this quantity of the carbonate has been increased and decreased as much as 50%.

With this undercoating of viscosity or water-carrying traits established in a degree of stability for smoothness, further advantage arises from incorporating an adhesive therewith. For commercial purposes, a low grade animal glue may be taken, and its proportion may be 13 3/4#, that is, in the quantity adopted for the ammonium bicarbonate. The glue, dissolved in the water, may have its plasticizing traits or properties increased hereunder by the inclusion of say 5 1/2# of sodium nitrate therewith. While these proportions for the adhesive, sodium nitrate, glue and water are suggested as 13 3/4# of the glue as to like quantity for the ammonium bicarbonate, such may vary with or away from the carbonate.

Furthermore, in this primary or undercoating, there may be adopted retaining traits against ready fracture. This tempering or water-carrying or retaining quality, which may even go to the extent of increasing the water-carrying or mixing values, is attained thru glycerine, which may be in the quantity of 51 1/2#. For such tempering agent, sulphonated oils, of which sulphonated castor oil may be preferred, may be adopted with the quantity in the range of 45#. There may even be variation up and down of 5% or more, as well as with the glycerine.

With this gum dispersed thru the carbonate and nitrate treated adhesive as a vehicle or carrier including the glycerine or tempering agent, there may be introduced the clay or kaolin, 265#, even with an additional 90# of water. The purpose had with this clay is that such may be the filler or body and be of fine particle size or texture. The quantity of water may have its variation for the desired degree of spreadability and be sufficient in the viscosity range for the ingredients, as for dip, spraying, brush painting or roll coating.

Upon pouring a charge of hot material into the container coated with the barrier or dam and having thereon for the film substance a resin, non-adhesive or differing from the traits of asphalt, the severance may result in approximately all of each of the coatings or residue thereof going with the container.

Example of film coating:

|                               |      |
|-------------------------------|------|
| Starch material               | 7#   |
| Plastic film-forming material | 7#   |
| Water                         | 200# |

When an additional or undercoating be desired, such may be

|                        |         |
|------------------------|---------|
| Kaolin                 | 265#    |
| Water                  | 90#     |
| Gum, as karaya         | 5 3/4#  |
| Carbonate, as ammonium | 13 3/4# |
| Glue                   | 13 3/4# |

and may have

|                             |         |
|-----------------------------|---------|
| Glycerine                   | 51 1/2# |
| Sodium nitrate              | 5 1/2#  |
| Pigment, as carbon black    | 8#      |
| Sodium benzoate             | 1%      |
| Tetra-sodium-pyro-phosphate | 1.3#    |

thinned with water to the consistency desired for applying.

The clay powder or undercoating in its nature is porous, as distinguished from the film-forming overcoating being impervious. Furthermore, the film-forming overcoating has a property of adherence. The interposition of the powder material undercoating thereby provides a support for the film-forming overcoating and hereunder is desirably sufficient in the proportions to isolate the film-forming overcoating from the wall, due to the continuity of the undercoating.

An instance of practical range for coverage, may be taken as to a container for asphalt. The area for one side, say of a ream of fiber board 24" x 36"—a total of 2880 sq. ft.—may have the clay add to the weight of the board as much as 10# to 25#. In practice this runs around 18#. The fiber board itself varies over quite a range, according to the volume of asphalt. For 10# of asphalt, the container wall may run .020" to .040", or say from 220# to 440# per ream. When the container is to carry 400# of asphalt, the fiber board thickness may run .050" to .100", or weigh from 560# to 1120# per ream. The clay undercoating for one side would thus run say 18# to the ream, whether for the thin or heavier fiber board. The film-forming overcoating would run 1# to 2# per ream.

The functioning in all instances is to the end that there is non-adherence and non-contamination between the material of the container and the container walls. In the practice hereunder, even from heat of the contents, the container wall is immune from or resistant to attack by the contents.

The water dispersed clay has such clay run in solids, say from 40% to 60%, in the suspension mixture, with ingredients in solution to provide adhesive properties in body and effectiveness, relatively minor as to the clay, but with the adhesive traits at least just sufficient to establish a bonding mounting for the clay. This is in reality only a temporary characteristic for the bonding or holding action and is possessed as the coating is at first applied. For speed advantage in manufacture, it has been found that this single undercoating has its continuity better established in two applications. These may be in relatively close succession to range for the total clay some 5# per 1000 sq. ft. of surface.

Immediately thereafter, and while this undercoating is still alive in its adherent property; that is, before any crumbling away has occurred; an overcoating is applied. This overcoating skin or film, in some practice may be complete for the job. However, more efficient results are achieved in association with the major volume undercoating. The traits of this film are continuity against rupture. Commercial advantages as developed

and may have

|                 |        |
|-----------------|--------|
| Tempering agent | 20# 75 |
|-----------------|--------|

hereunder extend not only to polyvinyl alcohol, but to celluloses of methyl cellulose type, proteins of casein and mazlein types. In getting away from the celluloses by the proteins toward gums, as gum arabic and gum tragacanth, the skin-developing body in the starch association brings therewith physical problems. A definite comparison is the fact that with methyl cellulose such may be used in sufficient quantity at  $\frac{1}{2}$ # per 1000 sq. ft. of surface. For comparable results as to the tough film and continuity, the experience is for up to 2# of the proteins and 5# and more of the gum.

The film or thin skin overcoating has physical strength for continuity and distortion by folding of the wall for inside or outside corner, as well as scoring. This holding trait and elasticity, not only are effective against its rupture in normal carton handling practice, but the undercoating is anchored against crumbling away from the wall. The overcoating sufficiently seals that its film strength allows of collapsed carton storage, even for months, and with evaporation as to the undercoating limited to thru the wall body, even when such wall be fiber, it is very materially retarded, and may be further slowed down by a waterproofing coating on the converse or outer side of a fiberboard wall. The characteristic of fluidity in applying the undercoating due to ammonium carbonate, may be in some measure taken care of by other carbonate, especially of the alkali type as sodium or potassium. In the selection of ingredients or materials, costs, as to efficiency, are factors controlling.

The course adopted by applicant has shown advantages in compensating for, or rather permitting volatilization, or some vapor escape. In those instances where the container is to take a charge as hot filled; that is, above the boiling point of water, as say hot asphalt at 300° F., entraining or trapping of the vapors would tend to produce blisters at or in the wall and foaming or voids in the contents. Herein, the starch and methyl cellulose or other solution of the overcoating film or skin, tends to pass off at the high temperature. This it is free to do thru the porous clay body of the undercoating. The undercoating adhesive is of such minor proportion as not to fill or seal the pores of the fiberboard. Accordingly, the vapors generated by the hot asphalt do not come back into the asphalt, but thru and from the clay body pass into, thru and from the fiberboard outer side, at a rate to avoid bubbling or foaming of the asphalt, and still so distributed in the fineness of exit ways as not to weaken the container wall. Flow of the asphalt is not to contact the wall inner side, for there is the inert clay barrier or wall.

With the container charged with the congealing asphalt, there is the physical strength of the fiberboard wall sufficient, at least at this setting stage for the contents, to hold the clay as a sort of partition or barrier between the asphalt and the fiberboard, even should the film have disintegrated. The body of the clay is sufficient, in this inter-asphalt-and-fiberboard compartment as to constitute a dam against attack of the fiberboard by the asphalt. As the asphalt congeals, the hardness of its solid state is sufficient reinforcement .05" to .10" thick that as 70 a drum it may have a capacity of up to 400# of

asphalt for such gauge of fiberboard. In such instance the clay may run from 5# to 7# per 1000 sq. ft. and the starch-methyl cellulose 1 $\frac{1}{4}$ # per 1000 sq. ft. in which the latter film coat is 5 60% methyl cellulose. The proportion has been used successfully with 5# of clay per 1000 sq. ft. for the undercoating and  $\frac{1}{2}$ # starch-methyl cellulose for 1000 sq. ft. for the overcoating. With the hot asphalt acting to vaporize or destroy the 10 film and adhesives of the character of gum or glue, there remains the undercoating relatively inert clay body as the barrier. In this embodiment, the absence of a moisture or water vapor barrier, efficiently permits a sort of vapor breathing to avoid any entrapment or void cluster regions. The coatings as applied are of fluidity 15 to be ready flowing mixtures or solutions, with entire absence of tacky or jelling characteristics. From the foregoing, the subject-matter disclosed 20 herein relates to a container wall comprising an outer layer of fibrous material and an inner dual coating layer impermeable to asphaltum, bonded to but severable from said fibrous layer, said inner dual coating layer comprising a first major body undercoating of water-dispersed clay and sufficient adhesive that this first undercoating 25 may isolate the second coating from the wall, and said second continuous lesser-body-carrying coating agent thereon of organic resin-like material, independent of emulsion with water, possessing 30 a characteristic for thin film spreading in direct water solution over the less thin first undercoating and with such cohesive consistency to maintain the clay as a dam effectually spacing the 35 film from the fibrous body throughout the extent of the wall during hot charging thereon of asphaltum, for wall severability thereafter from the solidified asphaltum. Importance resides in water solubility characteristics of methyl cellulose in its use with starch in providing the organic resin-like material of the second lesser-body-carrying coating.

It is to be noted that the coatings as effective 40 to retain asphalt and the like, have oil proof and grease proof resistant qualities. However, due to the use of water suspensions and solutions for carrier or spreadability traits in applying, there is some slight moisture present. The film and wall tend to slow up drying out. Somewhat different 45 rate is developed when hot charge of contents be introduced into the container. This speeded up drying out is a sort of exhaling from the container wall.

This application is a continuation-in-part of 55 my Patent 2,333,023 for Container wall.

What is claimed and it is desired to secure by Letters Patent is:

A container wall comprising an outer layer of 60 fibrous material and an inner dual coating layer impermeable to asphaltum, bonded to but severable from said fibrous layer, said inner dual coating layer comprising a first major body undercoating of water-dispersed clay and sufficient adhesive that this first undercoating may isolate 65 the second coating from the wall, and said second continuous lesser-body-carrying coating agent thereon of organic resin-like material of methyl cellulose and starch, possessing a characteristic for thin film spreading in direct water solution when applied over the less thin first undercoating.

WILLARD O. MANOR.